

# UNITED STATES PATENT OFFICE.

ROBERT H. HENEMIER, OF NEW YORK, N. Y.

## TIRE-VALVE ALLOY.

1,147,398.

No Drawing.

Specification of Letters Patent.

Patented July 20, 1915.

Application filed January 4, 1915. Serial No. 489.

To all whom it may concern:

Be it known that I, ROBERT H. HENEMIER, citizen of the United States, and resident of New York, in the county of New York and 5 State of New York, have invented certain new and useful Improvements in Tire-Valve Alloys, of which the following is a specification.

The object of my invention is a tire valve 10 alloy particularly adapted for economy in construction, great strength, power, and capable of resistance to the corrosive effects of water, oil and vulcanized rubber.

A further object of my invention is a 15 valve capable of being die cast. For an article of this character die casting results in great economy of manufacture. Heretofore it has been impossible, owing to the failure 20 of the metal used, to attain all the above functions.

In order to be air tight, the casting must be structurally dense. That is, it must have such a close grain when cast as to be free 25 from blow holes or pores,—not only to hold in the ordinary pressure of air within the tire but those extra pressures due to the sudden blows upon the tire when it strikes high points on the road.

Another requisite of my invention is that 30 it shall have tensile strength to withstand the pressures above referred to and to withstand the rough usage to which tire valves are subjected. With the metal heretofore used for die casting an ordinary wrench 35 would sever the valve when it was screwing the clamp nut into place. My die casting therefor must be in this respect and supply an article which has such tensile strength as to resist the destructive tendencies of 40 monkey wrenches. Such a die casting further must resist the corrosive action of water since it is so frequently and for such long periods exposed to the action of the elements. Furthermore, it must resist the 45 chemical action of air, and of oil which is apt to fall upon the valve either from the machine or from modern road beds. It must also resist the action of vulcanized rubber for it is rubber with which it is in 50 constant contact where it is attached to the wheel. A failure to meet this test results in leaks, and damaged valves and tubes. For this reason, my invention consists of a valve having any desired construction and composed of an alloy of aluminum

and nickel. Copper may be added to the alloy and improve its density and tensile strength. The nickel assists in protection from the elements and hardens it. The aluminum supplies light weight, ductility 60 and a binder for the other elements in the alloy. I preferably use between 5% and 15% of nickel, between 75% and 85% of aluminum, and between 7% and 10% of copper. The mixture of these amounts of 65 metal is made in the melting pot whence it is driven under pressure into dies adapted to mold the alloy into its final shape. This step of the process is well known in die casting.

By using the proportions of the metals as above set forth I secure an alloy which has all the properties necessary for successful use in a valve stem, particularly when used in a pneumatic tire. These proportions produce an alloy having sufficient density, tensile strength and workability so that the stem may be readily machined and when complete is impervious to air under pressure and will stand rough handling 80 without breakage or distortion.

What I claim is;

1. An alloy of aluminum, nickel and copper containing from about seventy-five (75) per cent. to about eighty-five (85) per cent. 85 of aluminum, about five (5) per cent. to fifteen (15) per cent. of nickel and from about seven (7) per cent. to ten (10) per cent. of copper.

2. As a new article of manufacture, a tire 90 valve stem composed of an alloy of aluminum, nickel and copper wherein the aluminum content composes the major portion thereof the aluminum content being less than 85%.

3. As a new article of manufacture, a tire valve stem composed of an alloy of aluminum, nickel and copper containing from about seventy-five (75) per cent. to about eighty-five (85) per cent. of aluminum, 10 about five (5) per cent. to fifteen (15) per cent. of nickel and from about seven (7) per cent. to ten (10) per cent. of copper.

Signed at New York in the county of New York and State of New York this 9th day of October A. D. 1914.

ROBERT H. HENEMIER.

Witnesses:

MYRON F. HILL,  
LOUIS MECKES.